

June 25, 1963

R. M. PARKE

**3,094,752**

## DIP FORMING TUBING

Filed Dec. 1, 1960



Inventor:  
Robert M. Parke,  
by James J. Lichelli  
His Attorney.

1

3,094,752

DIP FORMING TUBING

Robert M. Parke, Schenectady, N.Y., assignor to General Electric Company, a corporation of New York  
Filed Dec. 1, 1960, Ser. No. 73,069  
1 Claim. (Cl. 22—203)

This invention relates to dip forming tubing and more particularly to an improved method of dip forming a tubing about a central core with subsequent removal of the core.

Various methods, such as welding, casting or extruding, are utilized in present manufacturing practices, generally depending on the metal involved, to provide metallic tubing. In the manufacture of tubing from the harder metals, such as, iron and steel, the metal may be provided in the form of a sheet or strip which is rolled and continually welded in order to form a tube. Alternatively, tubes from such metals may be cast by well known casting processes. Of the softer metals, such as, aluminum, copper, lead, tin, etc., tubes may be formed by an extrusion process. This latter process may provide tubes of 25 to 50 feet in length and greater. However, the harder metals are quite difficult to extrude, the practicalities and economics of manufacture are very high, and thus resort is made to casting and welding. Those metals which are easily extrudable, the softer metals, are often limited in length because the apparatus employed must generally be as long as the effective lengths of the tubing. There are also practical and economic problems in both processes because of the necessity of starting with a solid preformed body. In either process, it is understood, that in order to provide a separate interior lining, for example, a noncorrosive one, separate or additional means is necessary, if feasible. It is thus very desirable to have an economical and practical process to provide tubing of short or long lengths from various metals, both the harder and softer metals and without the necessity of starting with preformed bodies and at the same time providing a lining therefor if desirable. It has been discovered that the inherent problems and difficulties as described may be overcome by the application of a dip forming process in tube manufacture.

Accordingly, it is an object of this invention to provide an improved method of producing tubing.

It is another object of this invention to provide an improved method of dip forming tubing.

It is still another object of this invention to provide an improved method of dip forming tubing of extensive lengths.

It is another object of this invention to provide an improved method of dip forming tubing with coated interiors.

Briefly described, this invention includes passing a wire, core or rod of a low temperature melting point material through a bath of a high temperature melting point material and regulating the rate of traversal of the core through the molten bath so that the high temperature melting point material solidifies on the core material in tube form, and thereafter the core or rod is removed from the tube by melting.

This invention will be better understood when taken in connection with the following description and the drawing in which:

FIG. 1 is a schematic representation of a process layout of a preferred form of this invention; and

FIG. 2 is a cross sectional and elevational view of a rod passing through a bath.

Ordinarily, it is well known in dip forming processes that a strip of a given metal, for example, steel, may be passed through a molten steel bath so that the molten

2

steel solidifies on the strip and the strip is therefore increased in size, or, that one metal, for example, iron, may be passed through a bath of a dissimilar metal, for example, zinc, to have a zinc coating solidified thereon.

5 Similar processes may be employed either for joining purposes as in tube manufacture or for increased wall section, etc. However, these processes relate to what may be described as a single occurrence process which provides a given coating to a given structure with the added coating remaining as an integral structure with the core to produce a final product. Serious consideration has been given to the dip forming process in tubing manufacture primarily because of appreciably diminishing the economic factor. As before stated, it is extremely difficult 10 to extrude, for example, harder metals as iron, steel, nickel, etc. in tube form and it is also difficult to provide extensive lengths of tubings from these and other such metals.

Accordingly, it has been discovered that metal tubings, 15 also of the harder metals, and of extensive lengths may be provided by means of an unique application of the dip forming process. Essentially this process includes passing a metal wire, rod or core, for example, silver, through a bath of, for example, iron, to provide a solidified iron 20 coating or tube on the silver core by dip forming process. Thereafter, the composite structure is heated just above the melting point of the silver so that the silver is liquefied and removed from the composite structure to provide an iron tube. A dip forming process and apparatus is the 25 subject of a copending application S.N. 530,283, Carreker, filed August 24, 1955, now U.S. Patent No. 3,008,201, and assigned to the same assignee as the present invention. The subject of this copending application is included by reference herewith and the apparatus used 30 therein is a preferred form of the apparatus and insofar as applicable, the stepwise process to be employed in the practice of this invention. Accordingly, FIG. 1 of this application, is similar to FIG. 1 of the aforementioned copending application.

40 Referring now to FIG. 1, there is illustrated a schematic representation of a dip forming apparatus of this invention as one working example. Exemplary materials to be described in relation to one working example are iron and silver, although it is to be understood that various 45 other combinations, such as, copper-steel, and others to be hereinafter described may be suitably employed. Silver has a melting point of about 960° C. and is readily available or easily produced in wire or rod form, but more particularly, represents no difficult problem in 50 extrusion because of its good ductile properties. Furthermore, silver may be readily and easily cleaned by well known chemical cleaning compositions, such as acid baths, etc. As illustrated in FIG. 1, an elongated silver wire 1 in a solid state having a first cross sectional configuration and area is continuously withdrawn from a storage means 2, such as, a reel or the like, and is guided by any appropriate means, such as, a sheath, pulley or drum 3 through preliminary treatment apparatus 4. Apparatus 4 in this instance includes a well known roll type 55 of straightening device for the silver wire 1. After traversing the straightener 4, the wire 1 proceeds into a conventional surface cleaning apparatus 5, for example, an electrolytic cleaning bath, and a rinsing or washing bath 6. The straightened, clean and wet wire 1 is then 60 guided by guide means 7, which is similar to guide means 3, into and through an elongated enclosure or tubular conduit 8. Conduit 8 includes a drying means 9, which may be supplied with a neutral atmosphere from a source 10, and conventional power driven feed rolls 11 which frictionally engage and drive wire 1 into a vacuum entrance 65 chamber 12. Chamber 12 is provided with a vacuum 70

source 13 which permits the wire to pass into chamber 12, but prevents the passage of atmosphere therewith. Wire 1 then proceeds into an entrance port 14 provided in the bottom of a crucible 15, and then passes through a bath of molten material, for example, iron, which is contained in crucible 15. The molten iron in crucible 15 accretes or deposits and solidifies upon and around the outer surface of silver wire 1 as a sheath or coating, increasing its cross sectional area appreciably, and providing an elongated and composite body 16 as best shown in FIG. 2.

Referring now to FIG. 2, wire 1 is illustrated as passing through entrance port 14 and through the molten bath of iron 17. Molten iron 17 commences solidifying on wire 1 adjacent the entrance port and continues to attach or solidify on wire 1 in increasing quantity until wire 1 has passed through the bath. The rate of deposition is of course dependent on the kind of metals employed together with their related melting points and more importantly on the rate of traversal of the wire 1 through the bath. Since dip forming, to apply steel on steel, lead on copper, tin on copper and zinc on steel, etc., is well known, the various design conditions for the practice of this invention are easily calculated or set up. Ordinarily, the requirements are that the metals have sufficiently different melting points commensurate with transit time in the bath, or rate of traversal therethrough, such that melting of the core material is substantially prevented. The temperature differential is not, however, the prime requisite. It is further defined by saying that the heat capacity of the core material must be sufficiently high so that the core material may take up or adsorb sufficient heat from the bath material to provide solidification of the bath material without melting of the core material. In a working example of this invention, a silver wire of about 1 inch to 1½ inches in diameter, at room temperature, may be fed through a molten bath of iron or steel at about 1570° C. With a rate of travel of about 25 to 300 feet per second or about a 1 second transit time, a ¼ to ½ inch coating is attained. A further working embodiment of this invention applies to the formation of copper tubing utilizing lead or tin as the wire or core material. Best results are obtained when the core material has been precleaned as described and where vacuum entry is employed.

After emerging from crucible 15, the silver-iron composite body is passed into a sizing apparatus, such as, a pair of sizing rolls 18. Apparatus 18 functions to remove or correct minor surface irregularities and provide the proper or predetermined O.D. In this respect, it is to be understood that shrinkage or contraction of the coating about the core material or wire introduces stresses in the coating which may lead to cracking. Such cracking is dependent on the various metal combinations employed, time-temperature conditions and the sizes or wall thicknesses of the final tube. These conditions may be prevented or minimized in marginal applications by providing surface variations in the core material so that contraction of the coating may be adsorbed by movement of the core material. Alternatively, the core material may be porous or hollow, etc. It is to be noted that a splined or corrugated core configuration may be employed to provide a resultant tubular configuration having internal projections or fins. Composite body 16 is guided by means of a temperature controlled duct conveyor 19, to any suitable receiving means, such as a reel 20, where it may be temporarily permitted to accumulate. Thereafter, the composite body 16 is withdrawn from receiving means 20 and passed through winding and cutting apparatus 21 whereby body 16 is suitably wound, or cut to length, and manually or automatically placed within a furnace 22 in order that the temperature may be raised sufficiently to melt the silver and the silver removed therefrom. Furnace 22 may be suitably combined with the same furnace utilized to melt the iron in crucible 15.

The resulting iron tube is removed as the final product as indicated by arrow 23.

From the foregoing, it may be readily understood that an apparatus is provided in which continuous casting or dip forming by accretion upon a length of core material provides an increased cross sectional material which may thereafter be processed into tubular form. One or more passes through bath 15 may be made depending on the final tube size desired. The composite body 16 also may be arranged in various configurations in furnace 22 to have molten silver flow therefrom by gravity, such as by having the composite body wound into a configuration similar to an "Archimedes" screw, or it may be rotated, or suitably moved to provide the same result. A connection is illustrated between furnace 22 and storage means 2 to indicate that the silver may be solidified and extruded in wire form for a repeat of the process, or to indicate closed circuitry where desired.

Two important advantages are to be gained by the practices of this invention. One of these important advantages is the production of tubes in an efficient and economic manner of those metals difficult to extrude and also a more economical production of ordinary tubing, such as for example, copper and the softer metals. In addition to the general practices of this invention, non-metals also may be employed as a core material together with other metals or non-metals. A unique example is the utilization of mercury in the frozen state to provide tubular configuration from metals or non-metals from which the mercury may be extracted at room temperature. In any instance, best results are obtained when the melting points of the materials are reasonably spaced with consideration of the heat capacity of the core material to avoid melting of the core material. A difference of about 300° C. is preferred for most metals.

The second important advantage in the process is the provision of a coating or lining in tubular configuration. In many industrial processes and in particular in food processing apparatus, there is required, or desired, extensive lengths of relatively low cost tubing having a preferred internal coating which is generally non-corrosive or which does not affect taste of the products flowing therethrough. The silver-iron combination provides a thin silver coating in an iron tube, and in the tin-copper combination, the process provides a tin coating on a copper tube. The coating or alloying, referred to as joining, is controlled first by the choice of materials used, i.e., where the materials are or are not capable of alloying with each other, and to what degree. The thickness of the lining or the extent of alloying may be controlled by controlling the rate of cooling of the composite structure 16 in temperature duct 19 after it leaves bath 15, with longer cooling periods providing increased thickness of coating or increased alloying.

In extensive operation a furnace 22 may be provided to replenish molten material in crucible 15 in order to maintain a predetermined level and uniform size of the composite body. Starting of the sequence is facilitated, for example, by employing a starting section of the core material of a material having a higher melting point than the bath material, or by suitable apparatus which will commence drawing wire 1 through crucible 15 at the entrance seal 14, or by a flying start process. The rod wire or core material of this invention may be an alloy as well as the bath material may be an alloy. Core alloys may be desirable for various purposes, for example, for increased strength such as, a copper lead alloy as a core material where lead alone would be too soft.

While a specific method and apparatus in accordance with this invention has been shown and described, it is not desired that the invention be limited to the particular description nor to the particular configurations illustrated, and it is intended by the appended claim to cover all modifications within the spirit and scope of this invention.

What I claim as new and desire to secure by Letters Patent of the United States is:

An improved method of forming tubular configurations of a given metal with an integral metal lining therein which comprises providing a molten metal bath of iron, providing an elongated core of a solid state metal taken from the class consisting of copper, silver, tin, aluminum, lead and nickel, passing the said core through the said bath in a dip forming process to provide a coating of iron on said core to form a composite body, thereafter passing 10 said composite body through a temperature controlled duct, controlling the rate of cooling of said composite body in said duct to in turn vary the coating action between said iron and said core providing a lining for said iron, and thereafter heating said composite body for melt- 15

ing and removal of the remainder of said core resulting in an iron tube with a core metal lining.

References Cited in the file of this patent

UNITED STATES PATENTS

|           |          |               |
|-----------|----------|---------------|
| 443,536   | Norman   | Dec. 30, 1890 |
| 1,396,918 | Brace    | Nov. 15, 1921 |
| 1,710,534 | Field    | Apr. 23, 1929 |
| 1,862,249 | Wilder   | June 7, 1932  |
| 2,123,894 | Hazelett | July 19, 1938 |
| 2,716,790 | Brennan  | Sept. 6, 1955 |

FOREIGN PATENTS

|         |               |               |
|---------|---------------|---------------|
| 817,048 | Great Britain | July 22, 1959 |
|---------|---------------|---------------|